

3,737,369  
**ALKALINE DIGESTION OF A MIXTURE OF COTTON LINTERS AND FIBROUS VEGETABLE MATERIAL AND PRODUCT THEREOF**  
Eduardo J. Villavicencio, Paramonga, Peru, assignor to Process Evaluation and Development Corporation, New York, N.Y.  
No Drawing. Filed Mar. 13, 1972, Ser. No. 234,362  
Int. Cl. D21c 5/00  
U.S. CL. 162—95 10 Claims

**ABSTRACT OF THE DISCLOSURE**

Alkaline digestion of a mixture of cotton linters, having a fiber length of about 2 to about 5 millimeters, and fibrous vegetable material.

This invention relates to methods of chemically pulping blends of diverse cellulosic materials. In particular it relates to a process for pulping blends or mixtures of cotton linters with the fibrous fraction of vegetable materials such as straw, flax, rice hulls, hemp, esparto, bamboo and other like materials, especially depithed sugarcane bagasse. The invention further relates to the resultant pulps and to paper products prepared therefrom.

Cotton linters (the staple left on cotton seeds after ginning) have previously been used to prepare paper pulp. The linters, which are approximately 90% or more pure cellulose, are normally pulped by mechanical pulping processes using, e.g., Hollander refiners and very small amounts of reactive chemical for oil and wax removal. Pulps have also been prepared by chemical pulping of the fibrous portions of straws, grasses and other like vegetable materials such as depithed sugarcane bagasse. Bagasse and similar vegetable material fibers have a relatively very high hemi-cellulose content (upwards of 28% by weight of the total lignocellulose material) a substantial proportion of which is retained after a conventional soda process pulping. Because of this characteristic bagasse pulps hydrate extremely fast and are typically observed to be (1) too easily refined, and (2) intrinsically weaker, especially in regard to tearing strength of paper made therefrom. Because of the very diverse nature of cotton linters and bagasse and like vegetable fibers and the pulping processes conventionally applied to each it has not previously been considered feasible to prepare paper pulps from blends of these materials.

In accordance with the present invention it has been found that blends or mixtures of 2 to 15 weight percent cotton linters and correspondingly 98 to 85 weight percent lignocellulosic fibers of vegetable materials such as sugarcane bagasse may be chemically pulped to produce pulps useful for the manufacture of paper. Preferably the amount of linters in the mixture is from about 5 to about 10 weight percent based on total weight. By blending the fibers before digestion xylosan (the major hemicellulose constituent of bagasse) is released from the bagasse and absorbed by the cotton linters during the alkaline digestion. The rate of hydration of the bagasse fibers is thus reduced and that of the cotton linters is increased. Pulp from the blend will take refining energy and yield paper having improved strength characteristics as compared to 100% bagasse pulp furnish.

It is an important and critical feature of the present invention that the cotton linters utilized have a maximum fiber length of not more than about 4 to 5 millimeters and a minimum fiber length of not less than about 2 to 2.5 millimeters. In trial runs of the process of this invention it has been observed that pulps including cotton linters fibers longer than the aforesaid maximum, e.g. about 6 millimeters cannot be satisfactorily refined; apparently be-

cause the linters agglomerate and become mechanically entwined into relatively thick ropes which plug the refiner. When the cotton linters used are shorter than about 2 millimeters the tear strength and tensile strength properties of paper made from the resultant pulp tend to decrease as compared to paper from pulps containing cotton linters of longer fiber length. Present experience indicates that the most preferred fiber length for the cotton linters is about 3 to 4 millimeters. Overlong cotton linter fibers may be reduced in size to a suitable length for use in practicing the invention by any suitable means. One particularly suitable method that has been satisfactory in trial runs has been through the use of commercially available Sprout-Waldron (Muncy, Pa., U.S.A.) rotary knife cutters, in particular the MRP model as fully described in that company's Bulletin 261.

Except for the presence of cotton linters the pulping process of this invention is otherwise the same as typical processes used for pulping of vegetable material fibers. Thus, the weight ratio of total lignocellulosic and cellulosic (i.e., cotton linters) materials (dry weight basis), to 20 digestion medium is between about  $\frac{1}{5}$  and  $\frac{1}{3}$  (e.g.,  $\frac{1}{4}$ ); the digestion temperature is from about 340° to about 380° Fahrenheit (e.g., 350° Fahrenheit) and the digestion time ranges from about 15 minutes to several hours or more, 25 depending primarily upon the specific lignocellulosic material being pulped. For pulping mixtures of linters and depithed sugarcane bagasse the digestion or "cooking" time is usually from about 15 to about 40 minutes, preferably 20 to 30 minutes. The pulping process may be combined with 30 a preliminary acid prehydrolysis step in which case alkaline cooking times can be reduced (for example, 5 to 20 minutes, preferably 10 to 15 minutes, for bagasse-linter blends). Any desired alkaline pulping chemicals may be used. Suitable chemicals are described, for example, in 35 Kirk-Othmer's "Encyclopedia of Chemical Technology," second edition, volume 16 (1968), beginning at page 702.

After digestion the pulp is refined, screened, washed, etc. in the usual manner prior to use as furnish to the 40 paper making machine.

The invention has been specifically demonstrated for 45 pulping of mixtures of cotton linters and sugarcane bagasse. However, it is not limited to bagasse as the lignocellulosic feed material, but is applicable as well to mixtures of cotton linters and fibers of vegetable materials such as bamboo, various straws, hemp, sisal and the like.

In the application of the invention to pulping of mixtures of linters and bagasse the bagasse fibers used should 50 be as pith-free as is reasonably possible. Suitable bagasse fiber feed materials may be prepared, for example, via the use of the apparatus and/or methods described in U.S. Pat. 3,537,142, issued Nov. 3, 1970 or in my prior co-pending U.S. Application Ser. No. 54,580, filed July 13, 1970 and now U.S. Pat. 3,688,345. For highest yields it 55 is preferred that the bagasse fiber feed material be one which has been subjected to a two-stage depithing operation, i.e., first "dry" depithed in accordance with the aforesaid U.S. Pat. 3,537,142 and then further "wet" depithed in the presence of at least about 4.5, normally from about 5 to about 10, parts by weight of water per part by weight of fiber (bone-dry basis) in accordance with the 60 said U.S. application Ser. No. 54,580; the entire disclosure of which is incorporated herein by reference.

The blend or mixture of cotton linters and the lignocellulosic fibers of vegetable material (such as bagasse) 65 may be prepared in any suitable manner and at any suitable time prior to commencement of the alkaline digestion. In one presently preferred embodiment the blend is formed by adding a water slurry containing the appropriate desired amount of linters to the above described second stage wet depithing operation on the bagasse fibers;

thus, in effect, forming the blend in the wet depithed. In this way it is possible to remove some of the greases and oils in and on the cotton linters as received and thereby improve the xylosan transfer from the bagasse to the linters in the subsequent alkaline digestion.

The proportions of the alkaline, preferably sodium, pulping chemicals used are all expressed in terms of their sodium oxide ( $Na_2O$ ) equivalent. Preferably the total  $Na_2O$  content of the digestion liquor is about 12 weight percent.

Practice of the invention is illustrated by the following specific but nonlimiting examples. In the examples the properties shown for the pulp and for paper samples prepared therefrom are all determined by standard TAPPI procedures. For example, the "K-number" of the pulps is the potassium permanganate number, a standard TAPPI test for determination of residual lignin. Tensile strength of the paper samples is the tensile breaking length, in meters, determined on an Instron tensile tester with a specimen 1-inch wide, 4-inches long (between test jaws) and at a jaw separation rate of 1-inch per minute.

In the following examples the lignocellulosic material to be pulped was depithed sugarcane bagasse prepared in the apparatus and with the method described in the aforementioned U.S. Pat. 3,537,142. All runs were made using a soda process cooking solution containing 12 weight percent (as  $Na_2O$ ) sodium hydroxide. All digestions ("cooks") were conducted at a ratio of about 4 parts by weight cooking liquor for each part by weight (dry weight basis) of the mixture of cotton linters and bagasse fibers or of these individual materials above in the comparative runs. The digestions were each performed for 30 minutes in a closed vessel at a steam pressure of 100 to 110 pounds per square inch gauge. After blowdown from the digester the pulps were cleaned, centrifuged, and washed in the usual manner. Thereafter, the beating or refining

times of the pulps to various Canadian Standard Freeness were determined and certain properties of papers prepared from the beat pulps were tested. For comparison purposes pulp was prepared from the same sugarcane bagasse fibrous material alone, and from the cotton linters alone, in the same manner as described above and properties of sample papers made from these pulps were also determined. Results are shown in the following Tables I, II and III.

TABLE I.—PULP RAW MATERIALS

| Weight percent of<br>solubles in— | Bagasse<br>fibers | Cotton<br>linters<br>(as re-<br>ceived) | Short cotton linters |      |      |
|-----------------------------------|-------------------|-----------------------------------------|----------------------|------|------|
|                                   |                   |                                         | #1 1                 | #2 1 | #3 1 |
| Cold water                        | 9.25              | 3.05                                    | 4.75                 | 4.43 | 4.92 |
| Hot water                         | 10.39             | 3.38                                    | 5.05                 | 4.60 | 5.63 |
| One percent $NaOH$                | 29.7              | 6.31                                    | 10.5                 | 10.4 | 11.4 |
| Alcohol/benzene                   | 4.0               | 1.52                                    | 2.99                 | 2.75 | 2.84 |

<sup>1</sup> The short cotton linters were prepared by size reduction using Sprout-Waldron rotary knife cutter, Model MRP with different screens—Short linters #1,  $\frac{1}{4}$  inch screen, fiber length 1.8 millimeters; short linters #2,  $\frac{1}{8}$  inch screen, fiber length 3 millimeters; short linters #3,  $\frac{1}{4}$  inch screen, fiber length 4 millimeters.

NOTE.—The linters as received had a fiber length of 8 millimeters. Attempts to use these in mixed material pulps were unsuccessful due to serious consistent plugging of the refiner.

TABLE II.—PULPING RUNS  
(All digestions with 12%  $NaOH$ )

|                                          |      | Run number |     |      |      |      |
|------------------------------------------|------|------------|-----|------|------|------|
|                                          |      | A          | B   | C    | 1    | 2    |
| Feed materials:                          |      |            |     |      |      |      |
| Bagasse fibers, percent                  | 100  |            |     |      | 90   | 90   |
| Cotton linters (as received),<br>percent |      | 100        |     |      |      |      |
| Short cotton linters:                    |      |            |     |      |      |      |
| #1, percent                              |      |            |     | 10   |      |      |
| #2, percent                              |      |            |     |      | 10   |      |
| #3, percent                              |      |            |     |      |      | 10   |
| Pulp yield, percent                      | 52.9 | 88.8       | 100 | 56.3 | 55.1 | 58.6 |
| Pulp K number                            | 24.5 | 1.5        | 1.7 | 17.8 | 20.4 | 21.4 |

TABLE III.—PHYSICAL PROPERTIES OF PAPER SAMPLES

| Beating<br>time<br>(minutes) | Canadian<br>Standard<br>Freeness<br>(milli-<br>liters) | Basis<br>weight<br>(ovendry,<br>grams per<br>meter) | Density<br>(grams per<br>cubic<br>centimeter) |                              |                 | Fold<br>number |
|------------------------------|--------------------------------------------------------|-----------------------------------------------------|-----------------------------------------------|------------------------------|-----------------|----------------|
|                              |                                                        |                                                     | Tear<br>factor                                | Tensile<br>break<br>(meters) | Burst<br>factor |                |
| Pulp from comparative run:   |                                                        |                                                     |                                               |                              |                 |                |
| A                            | 0                                                      | 860                                                 |                                               |                              |                 |                |
|                              | 8                                                      | 800                                                 | 63.1                                          | 67.0                         | 3,805           | 0.37           |
|                              | 16                                                     | 720                                                 | 62.6                                          | 64.0                         | 4,771           | 0.40           |
|                              | 24                                                     | 620                                                 | 61.6                                          | 60.5                         | 5,810           | 0.42           |
|                              | 32                                                     | 500                                                 | 62.1                                          | 53.6                         | 6,030           | 0.46           |
| B                            | 0                                                      | 900                                                 |                                               |                              |                 |                |
|                              | 60                                                     | 770                                                 | 61.1                                          | 341.8                        | 2,400           | 0.34           |
|                              | 75                                                     | 720                                                 | 59.6                                          | 320.0                        | 2,800           | 0.38           |
|                              | 90                                                     | 630                                                 | 58.2                                          | 292.3                        | 3,400           | 0.40           |
|                              | 105                                                    | 570                                                 | 59.2                                          | 274.6                        | 3,845           | 0.48           |
|                              | 120                                                    | 500                                                 | 59.2                                          | 259.6                        | 4,290           | 0.48           |
| C                            | 0                                                      | 870                                                 |                                               |                              |                 |                |
|                              | 60                                                     | 810                                                 | 59.6                                          | 76.8                         | 1,902           | 0.35           |
|                              | 75                                                     | 730                                                 | 59.6                                          | 100.0                        | 2,204           | 0.35           |
|                              | 90                                                     | 650                                                 | 59.6                                          | 119.4                        | 2,510           | 0.39           |
|                              | 105                                                    | 590                                                 | 59.6                                          | 108.0                        | 2,763           | 0.41           |
|                              | 120                                                    | 500                                                 | 60.1                                          | 94.6                         | 3,005           | 0.45           |
| Pulp from Example:           |                                                        |                                                     |                                               |                              |                 |                |
| 1                            | 0                                                      | 860                                                 |                                               |                              |                 |                |
|                              | 8                                                      | 830                                                 | 62.6                                          | 71.7                         | 3,482           | 0.36           |
|                              | 16                                                     | 770                                                 | 62.1                                          | 68.0                         | 4,260           | 0.39           |
|                              | 24                                                     | 660                                                 | 62.6                                          | 64.0                         | 5,059           | 0.40           |
|                              | 32                                                     | 560                                                 | 61.1                                          | 61.0                         | 5,550           | 0.46           |
|                              | 40                                                     | 460                                                 | 61.6                                          | 57.7                         | 6,102           | 0.50           |
| 2                            | 0                                                      | 870                                                 |                                               |                              |                 |                |
|                              | 8                                                      | 830                                                 | 62.1                                          | 78.7                         | 3,273           | 0.34           |
|                              | 16                                                     | 780                                                 | 63.1                                          | 74.0                         | 3,953           | 0.37           |
|                              | 24                                                     | 700                                                 | 61.1                                          | 71.0                         | 4,844           | 0.42           |
|                              | 32                                                     | 600                                                 | 61.1                                          | 69.0                         | 5,465           | 0.42           |
|                              | 40                                                     | 470                                                 | 60.6                                          | 66.0                         | 5,841           | 0.48           |
| 3                            | 0                                                      | 860                                                 |                                               |                              |                 |                |
|                              | 8                                                      | 810                                                 | 62.1                                          | 71.5                         | 3,273           | 0.34           |
|                              | 16                                                     | 770                                                 | 62.1                                          | 69.8                         | 3,484           | 0.37           |
|                              | 24                                                     | 660                                                 | 60.6                                          | 66.0                         | 4,093           | 0.38           |
|                              | 32                                                     | 560                                                 | 60.1                                          | 61.3                         | 4,510           | 0.41           |
|                              | 40                                                     | 450                                                 | 60.1                                          | 55.4                         | 5,174           | 0.45           |

Graphical plotting of the data shown in Table III above indicates that the pulps and paper samples have the representative properties shown in the following Table IV at equivalent Canadian Standard Freeness.

TABLE IV.—COMPARISON AT EQUIVALENT CANADIAN STANDARD FRENESS

| At Canadian Standard Freeness of 650 milliliters | Examples |       |       | Comparative runs |       |       |
|--------------------------------------------------|----------|-------|-------|------------------|-------|-------|
|                                                  | 1        | 2     | 3     | A                | B     | C     |
| Beating time.....                                | 25.0     | 28.0  | 25.0  | 22.0             | 80.7  | 90.0  |
| Tear factor.....                                 | 63.8     | 70.0  | 65.0  | 61.5             | 300.0 | 119.4 |
| Tensile break.....                               | 5,100    | 5,200 | 4,100 | 5,550            | 3,600 | 2,510 |
| Burst factor.....                                | 24.0     | 29.5  | 21.5  | 28.5             | 22.0  | 10.5  |
| At Canadian Standard Freeness of 500 milliliters |          |       |       |                  |       |       |
| Beating time.....                                | 36.7     | 38.6  | 36.5  | 32.0             | 120.0 | 120.0 |
| Tear factor.....                                 | 59.0     | 66.0  | 58.0  | 53.6             | 259.6 | 94.6  |
| Tensile break.....                               | 5,900    | 5,750 | 4,850 | 6,030            | 4,290 | 3,005 |
| Burst factor.....                                | 28.5     | 33.5  | 25.0  | 32.0             | 31.0  | 15.0  |

As seen from the foregoing examples the method of this invention provides a practical procedure for pulping a blend of diverse materials to yield pulps having a good combination of properties compared to pulps prepared from vegetable material fibers alone, e.g., bagasse fibers. In all examples, the beating times to equivalent Canadian Standard Freeness are greater than in Comparative Run A and tear strengths are increased. The overall physical properties of papers prepared from the pulps of all examples, especially Example 2, are good to excellent.

I claim:

1. Method for the production of pulp comprising digesting a mixture of 2 to 15 weight percent cotton linters having a fiber length of about 2 to about 5 millimeters and 98 to 85 weight percent fibrous vegetable material with an aqueous alkaline digestion solution and recovering the resultant cellulosic pulp.

2. Method as defined in claim 1 in which the cotton linters constitute from 5 to 10 weight percent of the mixture to be pulped.

3. Method of claim 2 in which the fiber length of the cotton linter is about 3 to 4 millimeters.

4. Method of claim 3 in which the digestion is conducted at steam gauge pressures of from about 100 to about 125 pounds per square inch for a period of from about 15 to about 40 minutes using a 12 percent aqueous solution of sodium hydroxide as the digestion solution.

5. Method of claim 1 in which the fibrous vegetable material is depithed sugarcane bagasse.

6. Chemical pulp produced by the method of claim 5.

7. In the process of chemically pulping fibrous vegetable materials with an alkaline digestion solution the improvement comprising mixing the said material with 2 to 15 weight percent of cotton linters having a fiber length of from about 2 to about 5 millimeters thereby increasing the pulp refining time and tear strength.

8. Process as defined in claim 7 wherein the cotton linters have a fiber length of about 3 to 4 millimeters.

9. Process as defined in claim 8 wherein the cotton linters are admixed in an amount of from about 5 to about 10 weight percent.

10. Paper produced from the chemical pulp of claim 6.

#### References Cited

##### UNITED STATES PATENTS

30 1,389,936 9/1921 Clapp ----- 162—95 X  
1,839,996 1/1932 Rose et al. ----- 162—95 X

S. LEON BASHORE, Primary Examiner

A. L. CORBIN, Assistant Examiner

35 U.S. CL. X.R.

162—96